

## UNITED STATES PATENT OFFICE

2,235,828

PREVENTION OF SEASON CRACKING OF  
BRASS

Cedric Arthur Vincent-Daviss and Harold L. Maxwell, Wilmington, Del., assignors to E. I. du Pont de Nemours & Company, Wilmington, Del., a corporation of Delaware

No Drawing. Application March 12, 1940,  
Serial No. 323,634

9 Claims. (Cl. 91—68)

This invention relates to a method of inhibiting corrosion and, more particularly, to prevention or inhibition of season cracking of brass articles.

Brass articles which have been formed by cold working or which for other reasons have internal stresses are subject to a phenomenon known as "season cracking." After a period of time which may vary depending upon conditions and upon the amount of internal strain present in the brass articles, the brass develops cracks or fissures. Such season cracking may develop in cleaned brass articles in storage or shipment prior to use or during use.

An excellent method for cleaning oxide and other undesirable or unsightly impurities or deposits from the surface of brass articles consists in washing them with a solution of alkali metal cyanide. It has, however, been found that brass articles thus washed in a cyanide solution generally are more subject to season cracking than those which have been washed by conventional methods, such as acid pickling and soap and water treatments.

An object of the present invention is to provide a method for inhibiting or preventing season cracking of brass articles. A further object is to provide a means for cleaning brass articles with cyanide solutions and to produce cleaned brass articles which have little or no tendency to develop season cracking. The present invention also includes brass articles of manufacture prepared by the herein described method.

As one method of practicing the present invention we may clean cold worked brass articles, for example, cold drawn brass articles, stampings, or the like in a solution of sodium cyanide containing 0.1 to 5 ounces of sodium cyanide per gallon. After the articles have been washed in the cyanide solution, while still wet, the brass surface is washed thoroughly with water by rinsing or spraying until cyanide is substantially completely removed. The brass articles then are wetted with a solution of an organic sulfur compound of the type described hereinafter. The articles are then dried so as to leave a film of the sulfur compound on the surfaces thereof.

The organic sulfur compounds which are suitable for practicing the present invention are the mercapto aryl thiiazoles, hydrocarbon mercaptans and their corresponding disulfides. Examples of these are: mercapto benzothiazole and its homologues such as the mercapto tolylthiazoles, mercapto xylithiazoles, mercapto ethylbenzothiazoles, and mercapto naphthothiazoles; also thio-

phenols, thiocresols, dimercapto benzenes, thiophthalanes, benzyl mercaptans, methyl benzyl mercaptans, cyclohexyl mercaptan; long chain alkyl mercaptans such as lauryl mercaptan, cetyl mercaptan and the like and the corresponding disulfides. We prefer to use mercapto benzothiazole as it is readily available, being a common rubber accelerator, and gives excellent results.

The present invention is not restricted to the use of cyanide for cleaning the brass articles. The organic sulfur compound may be applied to any brass surface which has been cleaned by any suitable process sufficiently to afford uniform direct contact between the brass surface and the sulfur compound. In order to obtain the desired inhibition of season cracking, it is necessary only to deposit on the brass surface a thin film of the sulfur compound. This may be done by any conventional method; we prefer to apply a solution of the sulfur compound on the surface of the brass and then evaporate off the solvent to leave a film of the sulfur compound thereon. A convenient method consists in immersing the brass articles in a dilute aqueous solution of the sulfur compound, for example, in a solution containing 0.01 to 1% by weight of mercapto benzothiazole and thereafter dry the brass article. Likewise, the solution may be applied by spraying, brushing or other conventional method. The organic sulfur compound may be dissolved in either aqueous or non-aqueous solvent or dispersed in a liquid substantially inert to the brass surface as a suspension or emulsion. Also, various known film-forming substances may be incorporated with the sulfur compound in the liquid composition applied to the brass. If the brass surface has been cleaned with a cyanide solution or other substance which tends to accelerate season cracking, the cyanide or other foreign material should be substantially completely removed from the brass before applying the organic sulfur compound.

The following examples illustrate the effect of mercapto benzothiazole in inhibiting the season cracking of brass:

## Example I

Brass shotgun shell heads were divided into two lots of 15 each and the lots were given different treatments, as follows:

| Lot    | Treatment                                           |
|--------|-----------------------------------------------------|
| A..... | Dipped in 2% aqueous solution of sodium cyanide.    |
| B..... | Dipped in 0.05% solution of mercapto benzothiazole. |

The samples of both lots were drained and dried in the air at room temperature. The samples then were stored in a moist atmosphere at a temperature of 120° F. for one month. The samples then were subjected to a standard mercury accelerated cracking test and examined for cracks. The following results were obtained:

| 10 | Lot | Treatment              | Percent cracked |
|----|-----|------------------------|-----------------|
| 15 | A   | Sodium cyanide         | 93.3            |
|    | B   | Mercapto benzothiazole | None            |

15 The above mentioned standard mercury cracking test was carried out as follows: The brass articles were etched, inside and out, with 40% nitric acid applied for a period of 15 seconds. After rinsing in water, a 1% solution of nitric acid containing 1% of mercurous nitrate was placed in the inside of the shells for 15 seconds. The shells then were again rinsed with water, wiped off and examined under a microscope at 75x magnification.

20 *Example II*

25 A lot of .22 caliber brass cartridge shells, which had been subjected to a conventional soap and water cleaning were dipped in a 0.05% aqueous solution of mercapto benzothiazole and dried at room temperature. The shells then were stored in a laboratory dessicator over 1% ammonia solution for 48 hours. Another lot of the soap and water cleaned shells, not treated with mercapto benzothiazole, were also stored 48 hours in a dessicator over 1% ammonia solution. Both lots then were subjected to the mercury cracking test described above, with the following results:

| Lot | Treatment              | Percent cracked |
|-----|------------------------|-----------------|
| A   | Mercapto benzothiazole | None            |
| B   | Not treated            | 80              |

30 *Example III*

35 Two lots of .22 caliber brass cartridge shells were dipped in sodium cyanide solution (2 oz. per gallon), rinsed in water to remove adhering cyanide and dried at room temperature. One lot was then dipped in a 0.05% solution of mercapto benzothiazole and dried. Both lots then were stored in a moist atmosphere for one month at 120° F. and for two weeks longer at room temperature. All samples of both lots then were subjected to the standard mercury cracking test, with the following results:

| 60 | Lot                                 | Treatment | Percent cracked |
|----|-------------------------------------|-----------|-----------------|
| A  | Treated with mercapto benzothiazole | 25        |                 |
| B  | Not treated                         | 95        |                 |

65 Our invention makes possible the storage or use of cold drawn brass articles for over long periods

of time without danger of excessive season cracking. The invention is useful for treating brass articles which are stored or used under conditions which ordinarily cause rapid season cracking. For example, we have found that brass articles treated by our invention are highly resistant to season cracking when stored in an ammonia atmosphere. The action of ammonia on brass articles is well known to accelerate the tendency to season crack.

10 We claim:

1. A process for cleaning brass articles which comprises washing said articles in a solution of alkali metal cyanide, washing to remove cyanide from the brass surface and depositing on the 1 washed brass surface an organic sulfur compound selected from the group consisting of mercapto aryl thiazoles, hydrocarbon mercaptans and the corresponding disulfides.

2. A process for cleaning brass articles which 2 comprises washing said articles in a solution of sodium cyanide, washing to remove cyanide from the brass surface, wetting the washed brass surface with a solution of an organic sulfur compound selected from the group consisting of mercapto aryl thiazoles, hydrocarbon mercaptans and the corresponding disulfides and drying to leave a 2 film of said organic sulfur compound on said brass surface.

3. A process for cleaning brass articles which 3 comprises washing said articles in a solution of sodium cyanide, washing to remove cyanide from the brass surface, wetting the washed brass surface with a solution of mercapto benzothiazole.

4. A process for cleaning brass articles which 3 comprises washing said articles in a solution containing 0.1 to 5 ounces of sodium cyanide per gallon, washing to remove cyanide from the brass surface, wetting the washed brass surface with a solution containing 0.01 to 1% by weight of mercapto benzothiazole and drying to leave a film of mercapto benzothiazole on said surface.

5. The method for inhibiting season cracking of a brass article which comprises depositing an organic sulfur compound to the surface thereof. 4

6. The method for inhibiting season cracking of a brass article which comprises coating the surface thereof with mercapto benzothiazole.

7. The method for inhibiting season cracking of a brass article which comprises applying to the 5 surface of said article a solution containing 0.01 to 1% by weight of mercapto benzothiazole and drying to leave a deposit of mercapto benzole on said surface.

8. A brass article which is resistant to season cracking, having deposited on the surface thereof an organic sulfur compound selected from the group consisting of mercapto aryl thiazoles, hydrocarbon mercaptans and the corresponding disulfides.

9. A brass article which is resistant to season cracking, having mercapto benzothiazole deposited on the surface thereof.

CEDRIC ARTHUR VINCENT-DAVIES. 6  
HAROLD L. MAXWELL.